# EUROPEAN PATENT SPECIFICATION

(11) **EP 0 464 013 B1**
(45) Date of publication and mention of the grant of the patent: **23.08.1995**
(21) Application number: 91850164.4
(22) Date of filing: 14.06.1991
(51) Int. Cl.: C21D 1/84, C22C 38/12

(54) **Steel and a steel manufacturing method**
Stahl und Verfahren zur Herstellung von Stahl
Acier et un procédé pour la fabrication d'acier

(30) Priority: 26.06.1990 SE 9002249
(43) Date of publication of application: 02.01.1992
(73) Proprietor: OVAKO STEEL AKTIEBOLAG, 813 00 Hofors (SE)
(72) Inventor: Lund, Thore, S-813 00 Hofors (SE); Drugge, Ing-Marie, S-813 00 Hofors (SE); Ingo, Anneli, S-712 34 Hällefors (SE)
(74) Representative: Karlsson, Leif Karl Gunnar

(56) References cited:
- EP-A- 0 349 023
- CH-A- 267 753
- US-A- 2 158 036
- US-A- 2 778 755

## Description

The present invention relates to a method of treating steel alloyed with molybdenum and/or tungsten to increase its mouldability/deformability to make it easier to mould or work before the final treatment thereof, e.g. by tempering. The present invention also relates to a steel of such composition treated by the inventive method and thereby having been provided with increased mouldability/deformability.

The method for increasing the mouldability of steel provided according to the invention comprises cooling a steel containing iron, carbon in an amount of from 0,1 to 1,15 %, and from 0,2 to 2,0 % of an alloying additive selected from the group consisting essentially of molybdenum, tungsten and mixtures thereof, at a rate whereat ferrite separates out in said steel before pearlite formation therein, said rate being less than about 80° C/s to form submicroscopic particles in the ferrite of metal carbide of the alloying additives. The steel prepared according to the invention is defined in claim 7.

According to a preferred aspect of the invention, said method can also be applied to a steel additionally containing chromium in an amount of between 1 and 2 % to increase its temperability.

The carbon content of steel in accordance with the invention is preferably within the interval 0,10 - 1,20 %, the intervals of 0,10 - 0,35 %, 0,25 - 0,60 %, 0,45 - 0,85 % and 0,70 - 1,15 % being suitable for casehardening steel, toughened steel, induction hardening steel and spring and roller bearing steel, respectively. The intentional additive (molybdenum and/or tungsten) is preferably present in the steel in an amount within the interval 0,2 - 2,0 %. In certain special situations, such as products requiring high temperability, the steel in accordance with the invention, is also, alloyed with chromium, the chromium-content being 1 - 2 %. Other alloying elements normally used in steel, such as silicon, manganese, nickel, vanadium and (with the exception of the special situation discussed above) also chromium, are limited to the lowest possible levels for the industrial manufacturing process used to produce the steel. Such steel is particularly useful for stressed structural members, particularly structural members requiring high ductility and fatigue-resistance. The amount of silicon and manganese in particular should be kept low, the total content of silicon and manganese being preferably less than 0,30 %, and the content of each of the elements silicon and manganese being preferably less than 0,15 %.

The steel treated in accordance with the invention may, for instance, contain the following elements when based on scrap steel:

| Si | Mn | P | S | Ni | Cu | Al |
|---|---|---|---|---|---|---|
| 0,10 % | 0,20 % | 0,015 % | 0,015 % | <0,10 % | 0,20 % | 0,010-0,060 % |

Such steel often contains 0,45 % molybdenum and 0,75 % carbon, and higher contents of molybdenum or carbon of course can be added if desired. Other "normal" remainder elements include 0,05 % silicon and 0,10 % manganese.

The method according to the invention thus comprises selecting a steel within the scope specified above, e.g. steel having an elementary composition in the range disclosed in EP-A1- 0 349 023, and subjecting it to cooling, the cooling rate being below a certain value as discussed in more detail below.

The steel prepared according to the inventive method is characterized by a ferrite phase containing a considerable amount of submicroscopic particles of the metal carbide type. A steel manufactured in accordance with the invention thus contains an unexpectedly high quantity of ferrite which makes it less hard to work.

The invention is most easily illustrated with reference to an eutectoid steel. As is known, an eutectoid steel, such as carbon steel containing 0,8 % carbon, has by definition a pearlite content of 100 % and is therefore difficult to mould/work regardless of how it has been allowed to cool. However, by means of the invention, a phenomenon appears which is particularly evident when the steel selected according to the invention has a composition close to eutectoid and is subjected to the cooling described. The phenomenon is that ferrite is surprisingly separated out first and a degenerated pearlite is then formed. The structure as a whole would normally be expected to be pearlite in character since the steel composition has substantially an eutectoid composition. Due to the ferrite having been separated out, the steel becomes less difficult to work/mould.

With an eutectoid steel having the prescribed composition and a molybdenum content of 0,50 %, a structure can be obtained through the invention which is similar to that of a carbon steel with 0,2 % carbon, i.e. a large portion of ferrite is separated from the pearlite. Such a structure is surprising for a steel having an eutectoid composition. In the structure obtained through the invention the pearlite is degenerated. Such degenerated pearlite is known per se and is typical for steel containing molybdenum.

The invention can be generalized as follows, with respect to an eutectoid steel composition. The following is required in order to obtain pro-eutoctoid ferrite in steel with nominally eutectoid composition:
1) The steel must contain a considerable proportion of a substance strongly prone to forming carbides. Examples of such substances are molybdenum and tungsten. The effect of adding a substance strongly prone to forming carbides is that the forming of pearlite is greatly delayed.
2) The steel must be substantially free from substances facilitating the formation of pearlite. Particularly, the amounts of silicon and manganese must be kept low.
3) Cooling must take place below a certain critical cooling rate if pro-eutectoid ferrite is to be separated out.

The critical cooling rate is determined by the composition of the steel, particularly by the amount of substance strongly prone to forming carbides. The quantity of ferrite separated out increases the lower the cooling rate. The quantity of ferrite separated out increases with increasing amounts of molybdenum or tungsten, and decreases with increasing amounts of silicon and manganese. The ferrite formed contains a considerable amount of submicroscopic particles of MC type. For a steel alloyed with only molybdenum, the carbides are molybdenum carbides. These carbide separations are typically 1 nanometer in size.

Although the invention most easily is described with reference to steel of eutectoid character, it will be understood that it can be applied with advantage to non-eutectoid steels suitable for use as e.g. case-hardening steel, toughened steel, induction hardening steel and spring and roller bearing steel.

The sulfur content in the steel may be adjusted depending upon the field of application of the steel. The sulfur content is suitably less than or equal to 0,015 % for steel which is intended for plastic molding as the primary molding operation. The sulfur content may be within the interval 0,010 - 0,025 % for steel which will primarily be subjected to cutting. If the demands on cuttability of the steel are high, the sulfur content should suitably lie within the interval 0,010 - 0,080 %.

The titanium content in the steel is suitable less than 55 ppm, and the oxygen content is suitable less than or equal to 20 ppm.

Other features and advantages of the present invention will become apparent from the following description of the invention which refers to the accompanying drawings.

Figure 1 shows a CCT diagram illustrating the invention.

Figure 2, 3 and 4 show, on three different scales of enlargement, the structure of a steel having a composition according to the invention after cooling.

Figures 5, 6 and 7 show, on the same enlargement scales as in figures 2 - 4, the structure of a carbon steel containing 0,2 % carbon cooled at the same cooling rate.

Figure 8 shows the structure of a steel produced according to the invention, but having a high molybdenum content and low silicon and manganese contents.

Figures 9 and 10 show the structure of steel coooled at the same rate as the steel according to figure 8, but having low molybdenum and manganese contents and a high silicon content (fig. 9); and a low molybdenum content and high silicon and manganese contents (fig. 10).

Numbers are shown for each cooling curve at the bottom of figure 1, which relate to the magnitudes of parameters stated in the middle of the rows in the table. Figure 1 refers to a eutectoid steel containing 0,5 % molybdenum and remainder contents below the limits specified above.

"Diameter/mm" refers to a comparison dimension for the cooling, i.e., the cooling rate for the curve in question is that obtained when air cooling a steel rod with the stated diameter in millimeters. "C/s (800-400)" refers to the cooling rate in °C per second in the temperature interval 800 - 400°C. "Ps/C" refers to the temperature in °C at which pearlite starts to form. "Hv (30 kg)" refers to the result of a Vickers hardness test with a load of 30 kg.

Figure 1 shows the area in which pearlite develops, marked with "P", between two generally horizontal lines defining the commencement and termination of the pearlite development. The pearlite amount of the structure is stated as a percentage close to the lower horizontal line for each cooling rate.

A wedge-shaped area exists in the upper part of Figure 1, above the upper pearlite limit curve. This wedge-shaped area is provided with the marking "F" and illustrates the ferrite development according to the invention. Figure 1 clearly shows that ferrite F starts to develop when the cooling rate is below 0,74 °C/s. Ferrite development can in fact be traced even at a cooling rate of 0,84°C/s, but the quantity of ferrite is slight. In practice, therefore, the cooling rate should be less than 0,80°C/s for the steel referred to in figure 1, i.e., a eutectoid steel which, besides iron and carbon, consists of 0,5 % molybdenum, 0,10 % silicon and 0,20 % manganese, whereas the remaining substances have the remainder contents stated above, as acceptable for ball bearing steel based on scrap.

It will be apparent that molybdenum may be replaced by tungsten or that tungsten may be added, in which case the range 0,2 - 2,0 % represents the total amount of molybdenum and tungsten, and the other alloying materials, particularly silicon and manganese are limited in the manner specified above and to the extent suitable for the manufacturing process used to make the steel. Similarly, more chromium may be added to increase the temperability of the steel.

Figures 2 - 4 illustrate that the steel described in connection with figure 1, cooled at a rate of approximately 0,21°C per second, acquires a structure fully comparable with the structure of pure carbon steel with 0,2 % carbon which has been cooled at the same rate and is illustrated in figures 5 - 7, respectively.

This comparison shows that a molybdenum or tungsten steel with a eutectoid composition, selected and treated according to the invention, will acquire a structure with a pronounced quantity of free ferrite, the ferrite quantity corresponding to that occurring in carbon steel with 0,2 % carbon, and the eutectoid steel produced according to the invention will therefore have a moldability/workability comparable to that of a carbon steel with 0,2 % carbon. However, it should be clear that the same effect is obtained, at least to a certain extent, for other steels and cooling rates within the prescribed limits.

Figure 8 shows the structure of a steel with 0,5 % molybdenum, approximately 0,30 % silicon, and less than 0,15 % manganese, obtained according to the invention.

Figure 9 shows the structure of a steel with 0,2 % molybdenum, approximately 0,30 % silicon, and less than 0,15 % manganese, said structure having been obtained at a cooling rate corresponding to that for the steel according to figure 8.

Figure 10 shows the resultant structure when the molybdenum content is low, i.e. 0,2 %, the manganese content is high, i.e. 0,30 % and the silicon is high, i.e. 0,30 %.

Figures 8 - 10 indicate that the desired favorable structure (figure 8) with a relatively large amount of free ferrite is primarily obtained when the steel composition has a molybdenum content within the interval 0,2 - 1,0 % and low contents of silicon and manganese (the other remainder contents being low as described above,) and when the steel is cooled at a rate lower than the critical value described in conjunction with figure 1.

It will be understood with reference to figure 1 that if a lower molybdenum content is chosen for the steel, a lower cooling rate is required if the ferrite development indicated in figure 1 is to be maintained. The greater the amounts of remainder substances, particularly silicon and manganese, contained in the steel selected, the less ferrite will be formed.

The ferrite developed in the structure is relatively "pure" since all elements which become deposited in ferrite are suppressed in the steel selected. The magnitude and purity of the ferrite phase thus offers good workability for the steel. The elements which give the final product its desired final properties, appear in the form of carbides and are released only when required, i.e., when the steel is tempered.

The submicroscopic particles separated out during the formation of ferrite are relatively uniformly distributed in the steel. Their distribution and their extremely minute size are not detrimental to the moldability of the steel and the carbon and carbide-builders (e.g. Mo) bonded in the submicroscopic carbides facilitate tempering of the steel due to quicker homogenization at austenitizing.

## Claims

1. A method for increasing the mouldability of steel prior to final treatment thereof, **comprising** the step of cooling a steel containing iron, carbon in an amount of from 0,1 to 1,15 %, and from 0,2 to 2,0 % of an alloying additive selected from the group consisting essentially of molybdenum, tungsten and mixtures thereof, at a rate whereat ferrite separates out in said steel before pearlite formation therein, said rate being less than about 80° C/s to form submicroscopic particles in the ferrite of metal carbides of the alloying additives.

2. The method of claim 1, **wherein** said steel additionally comprises from 1 to 2 % of chromium to increase its temperability.

3. The method of claim 1 or 2, **wherein** carbon present in an amount of between 0,1 and 0,35 %.

4. The method of claim 1 or 2, **wherein** carbon present in an amount of between 0,25 and 0,60 %.

5. The method of claim 1 or 2, **wherein** carbon present in an amount of between 0,45 and 0,85 %.

6. The method of claim 1 or 2, **wherein** carbon present in an amount of between 0,7 and 1,15 %.

7. A steel prepared by the method of claim 1 to 6, **comprising** ferrite containing a considerable amount of submicroscopic particles of the metal carbide type.

8. The steel of claim 7, **wherein** said particles have a typical size of 1 nanometre in case of molybdenum carbide.

## Patentansprüche

1. Verfahren zur Verbesserung der Formbarkeit von Stahl vor dessen Schlußbehandlung, umfassend die Stufe des Abkühlens eines Stahls, der Eisen, Kohlenstoff in einer Menge von 0,1 bis 1,15 % enthält und 0,2 bis 2,0 % eines Legierungszusatzes, ausgewählt aus der Gruppe, bestehend im wesentlichen aus Molybdän, Wolfram und aus Gemischen davon, enthält, mit einer Geschwindigkeit, bei der sich Ferrit in dem genannten Stahl vor der Pearlitbildung darin abscheidet, wobei die genannte Geschwindigkeit weniger als etwa 80 °C/sec beträgt, um in dem Ferrit submikroskopische Teilchen von Metallcarbiden der Legierungszusätze zu bilden.

2. Verfahren nach Anspruch 1, bei dem der genannte Stahl außerdem 1 bis 2 % Chrom umfaßt, um seine Anlaßfähigkeit zu verbessern.

3. Verfahren nach Anspruch 1 oder 2, bei dem Kohlenstoff in einer Menge zwischen 0,1 und 0,35 % vorhanden ist.

4. Verfahren nach Anspruch 1 oder 2, bei dem Kohlenstoff in einer Menge zwischen 0,25 und 0,60 % vorhanden ist.

5. Verfahren nach Anspruch 1 oder 2, bei dem Kohlenstoff in einer Menge zwischen 0,45 und 0,85 % vorhanden ist.

6. Verfahren nach Anspruch 1 oder 2, bei dem Kohlenstoff in einer Menge zwischen 0,7 und 1,15 % vorhanden ist.

7. Stahl, hergestellt durch das Verfahren nach Anspruch 1 bis 6, umfassend Ferrit, der eine beträchtliche Menge submikroskopischer Teilchen vom Metallcarbidtyp enthält.

8. Stahl nach Anspruch 7, worin die genannten Teilchen eine typische Größe von 1 nm im Falle von Molybdäncarbid aufweisen.

## Revendications

1. Procédé destiné à accroître l'aptitude au moulage de l'acier avant son traitement final, comprenant l'étape consistant à refroidir un acier contenant du fer, du carbone dans une quantité allant de 0,1 à 1,15 %, et de 0,2 à 2,0 % d'un additif d'alliage choisi dans le groupe constitué essentiellement par le molybdène, le tungstène et leurs mélanges, à une vitesse à laquelle le ferrite se sépare de l'acier avant la formation de perlite, cette vitesse étant inférieure à environ 80°C/seconde pour former des particules sous-microscopiques dans le ferrite des carbures de métal des additifs d'alliage.

2. Procédé selon la revendication 1, dans lequel l'acier comprend de plus de 1 à 2 % de chrome pour augmenter son aptitude à la trempe.

3. Procédé selon la revendication 1 ou 2, dans lequel le carbone est présent dans une quantité allant de 0,1 à 0,35 %.

4. Procédé selon la revendication 1 ou 2, dans lequel le carbone est présent dans une quantité allant de 0,25 à 0,60 %.

5. Procédé selon la revendication 1 ou 2, dans lequel le carbone est présent dans une quantité allant de 0,45 à 0,85 %.

6. Procédé selon la revendication 1 ou 2, dans lequel le carbone est présent dans une quantité allant de 0,7 à 1,15 %.

7. Acier préparé par le procédé selon les revendications 1 à 6, comprenant du ferrite contenant une quantité considérable de particules sous-microscopiques du type carbure métallique.

8. Acier selon la revendication 7, dans lequel les particules ont une taille typique de 1 nanomètre dans le cas du carbure de molybdène.
